

Patented May 22, 1928.

1,670,826

# UNITED STATES PATENT OFFICE.

AUGUST E. SCHUTTE, OF NORTHBORO, MASSACHUSETTS.

CONSTRUCTION OF SURFACINGS FOR ROADWAYS, SIDEWALKS, AND THE LIKE.

No Drawing.

Application filed December 16, 1925. Serial No. 75,868.

My invention relates to the upper course or wearing surface of pavements, sidewalks, floors and the like and particularly to that type which is composed of bitumen cementing mineral aggregate and having its cementing value augmented with reinforcing fibre. I have been granted a U. S. Patent No. 1,265,259 dated May 7, 1918 for the use of asbestos fibre for this purpose, but I have found that the asbestos supply is located principally in Canada, practically restricting the use of it to areas close to the source of supply on account of the great weight and therefore costly freight on the material. I have now found that vegetable fibres such as jute, cotton, etc., if specially prepared, treated and handled according to my method can be used as an admixture to bitumen without destroying the usefulness of the fibre through heat.

tically the same result. To practice my invention, I procure burlap waste for example such as bags, put them through a vat or tank containing asphalt of the proper penetration, eliminate the excess of asphalt by putting the material through a set of rolls or other squeezing device and then allow the thus saturated material to enter a cutting machine which is heated and which has, as its principal element, a series of rotating knives which will cut the material into fibres about  $\frac{1}{4}$ " in length or even longer if it is desired. This cut fibre is then allowed to enter the asphalt in the mixing plant and is then, with the asphalt, put into an appropriate mixer and there mixed with a suitable mineral aggregate. It can then be handled in the usual manner, raked and rolled upon the foundation, which is to receive and retain it.

Numerous attempts have been made to use vegetable fibre as an ingredient in bituminous pavements, but usually such fibre was destroyed through heat or made brittle and useless during the process of the manufacture of the wearing surface. Furthermore, it was found that the comminution and separation of such fibre was a difficult matter, requiring costly machinery and producing a material which will, instead of mixing through the whole mass, become balled and bunched, making it impossible to produce a homogeneous mixture with the bituminous cement.

The fibre being saturated with the bituminous cement cuts with a surprising ease, obviating all matting and tangling and gives a most excellent material for the reinforcement of the bituminous cement. It does not shorten or change either ductility, adhesiveness or cohesiveness of the cement, but augments every one of these qualities. It changes some of the cohesive properties into adhesiveness by saturating the individual fibre, the frayed ends of which have a larger contacting area with the mineral aggregate than if the fibre was not present. The fibre being first saturated seems to withstand all the temperatures consistent with laying the surface.

I have discovered that woven fibre such as burlap bags, cotton rags, etc., if they are first saturated and impregnated with a bituminous compound, can without balling or bunching easily be separated and cut up and mixed with the hot bituminous cement which forms a cementing medium for the aggregate.

In describing my invention I will speak of its use for construction of roadways and will confine myself to the use of old burlap bags although it is applicable to other fibrous materials for it is obvious that other fibrous materials from other sources can be used in exactly the same manner.

It is a well known fact that burlap bags or other rags are an article of commerce procurable anywhere thus the high freight problem is entirely eliminated. Vegetable fibre, having less than half the specific gravity of asbestos, can be used in great deal smaller quantities and produce prac-

80  
85  
90  
95  
100  
105  
110

In describing the use of my compound I have not described the proportions of the various materials, as in general these are well known to those skilled in the art. It is well known that in making a pavement compound there may be variations in the proportions of bituminous cement to mineral aggregate according to circumstances. When my compound above described is used it should be considered as a part of the bituminous cement in making the formula for a given piece of pavement and the amount of fibrous material used may depend on the wear to which the pavement may be put and to other conditions which those skilled in the art will understand.

What I claim as my invention is:—

1. A method of producing a paving material which comprises first saturating vegetable fibre with a bituminous cement, then

cutting the fibre into small particles and mixing it with bituminous and mineral material.

2. A method of making a bituminous pavement composition which comprises adding to a vegetable fibre a bituminous compound whereby the fibre will absorb the compound, then allowing the product to

cool, comminuting the mass, mixing mineral aggregate therewith and then mixing the whole with a bituminous cement.

3. A pavement comprising a mineral aggregate cemented with evenly distributed comminuted vegetable fibre impregnated with bitumen.

**AUGUST E. SCHUTTE.**